

# United States Patent [19]

Philip, Jr.

[11] Patent Number: 4,578,347

[45] Date of Patent: Mar. 25, 1986

[54] SUPERSENSITIZATION OF SILVER HALIDE EMULSIONS

[75] Inventor: James B. Philip, Jr., St. Paul, Minn.

[73] Assignee: Minnesota Mining and Manufacturing Company, St. Paul, Minn.

[21] Appl. No.: 645,344

[22] Filed: Aug. 29, 1984

[51] Int. Cl.<sup>4</sup> ..... G03C 1/02

[52] U.S. Cl. ..... 430/572; 430/570;

430/576

[58] Field of Search ..... 430/572, 570, 576, 584,  
430/601, 610

## [56] References Cited

### U.S. PATENT DOCUMENTS

|           |         |               |       |         |
|-----------|---------|---------------|-------|---------|
| 3,644,530 | 2/1972  | Bloom et al.  | ..... | 430/240 |
| 3,695,888 | 10/1972 | Hiller et al. | ..... | 96/123  |
| 4,003,746 | 1/1977  | Bigelow       | ..... | 430/601 |
| 4,346,154 | 8/1982  | McLaen et al. | ..... | 430/610 |
| 4,411,985 | 10/1983 | Morrow et al. | ..... | 430/610 |

### FOREIGN PATENT DOCUMENTS

|         |        |                |       |         |
|---------|--------|----------------|-------|---------|
| 1066261 | 4/1967 | United Kingdom | .     |         |
| 195872  | 7/1967 | U.S.S.R.       | ..... | 430/601 |

### OTHER PUBLICATIONS

"Effect of Some Phenyl Derivatives of the Elements of

the V Group of Periodic Table on the Photographic Properties of Sensitized Emulsions", (1967), M. A. Akhmedzyanov, V. I. Slesareva, M. S. Khaikin and S. A. Lerner.

"Investigation of Some Aryl Phosphines as Activators of Spectral Sensitization", (1969), M. A. Akhmedzyanov, S. A. Lerner, I. P. Sotnikova, A. S. Fakhruidinov and S. G. Fatanyants.

"The Relative Affinities of Co-ordinating Atoms for Silver Ion, Part II Nitrogen, Phosphorus, and Arsenic", Sten Ahrland, J. Chatt, N. R. Davies and A. A. Williams, Journal Chemical Society, 1958. Chemical Abstracts, p. 410, vol. 94, 1981.

Primary Examiner—J. Travis Brown  
Attorney, Agent, or Firm—Donald M. Sell; James A. Smith; Mark A. Litman

[57]

### ABSTRACT

The addition of water-soluble triaryl compounds selected from the group consisting of phosphines, amines, arsines, bismuthines and stibylidynes provides sensitizing effects and, when added to spectrally sensitized emulsions, provides a supersensitizing effect. The activity of these compounds is additive with other supersensitizers.

25 Claims, No Drawings

## SUPERSENSITIZATION OF SILVER HALIDE EMULSIONS

### BACKGROUND OF THE INVENTION

#### 1. Field of the Invention

This invention relates to the use of supersensitizers in photographic emulsions.

#### 2. Background of the Art

In most uses of silver halide in photographic materials, it is desirable to increase the speed or sensitivity of the emulsion. There are a number of different techniques for increasing the speed of an emulsion which are usually classified as chemical sensitization or spectral sensitization. Chemical sensitization usually involves modification of the silver halide grains to make the most efficient use of the radiation that they absorb. The three general types of chemical sensitization are sulfur sensitization, reduction sensitization, and precious (noble) metal sensitization. These methods of chemical sensitization are well known and firmly established in the art (e.g., James, T. H. and Vanselow, W. "Chemical Sensitization", J. Photo. Sci. 1, 133 (1953), Freiser, H. and Ranz, E., Ber der Bunsengesellschaft, 68, 389 (1964), and Pouradier, J. "Chemical Sensitization", Photographic Theory: Liege Summer School, A. Hautot, p. 111, Focal Press (London) 1963).

Spectral sensitization enables grains to benefit from radiation in regions of the electromagnetic spectrum where the silver halide would ordinarily not absorb. Dyes which absorb radiation and can transfer energy to the grains to help in the photoreduction of silver ions to clusters of silver metal are conventionally used to effect spectral sensitization.

Another phenomenon associated with the use of spectral sensitizing dyes is known in the art as supersensitization. The addition of small amounts of other substances, frequently in quantities of about one percent of the molar amount of the dye, can increase the spectrally sensitized speed of the emulsion by more than an order of magnitude. Some supersensitizers are dyes themselves, but many others do not absorb radiation in significant amounts in the visible portion of the electromagnetic spectrum. Therefore, the effect of supersensitizers on spectral sensitization is not clearly dependent on the ability of compounds to absorb radiation in the visible portion of the spectrum. Certain cyanines, merocyanines compounds analogous to cyanines, certain acyl-methylene derivatives of heterocyclic bases, and ketone derivatives such as p-dimethylaminobenzalacetone are known supersensitizers. Not all supersensitizers work with all spectral sensitizers. There is no general knowledge in the art that supersensitizers are capable of sensitization in the absence of spectral sensitizers. An expanded selection of supersensitizers is therefore desired.

Triphenylphosphine,  $P(C_6H_5)_3$  (hereinafter TPP), is reported in the literature as a supersensitizer for infrared sensitive silver halide emulsion using certain spectral sensitizing dyes (Zhurnel Nauchnoi i Prikladnoi Fotografi i Kinetografii 14 (2) 148-149 (1969) and 12 (6), 462-463 (1967), M. A. Akhmedyanov et al. and Zh. Prikl. Spektrosk., 1980, 33 (3), 557-56 M. I. Demchuk et al.). The use of triphenylphosphine presents a number of problems because it is insoluble in water and causes dramatic variations in infrared sensitivity over moderate periods of time during coating operations.

### BRIEF DESCRIPTION OF THE INVENTION

Water-soluble derivatives of triaryl phosphides, amines, arsenides, antimonides and bismuthides have been found to act as supersensitizers to spectrally sensitized and especially infrared spectrally sensitized silver halide emulsions and also to act as sensitizers for silver halide emulsions without spectral sensitizers.

These water-soluble supersensitizers have been found to be particularly effective in combination with other photographic adjuvants such as phenylmercaptotetrazole, poly(ethylacrylate) and the supersensitizer leucophor BCF.

### DETAILED DESCRIPTION OF THE INVENTION

Triaryl phosphides, arsenides, antimonides, and bismuthides wherein at least one aryl group has a substituent which renders the compound water-soluble are supersensitizers for spectrally sensitized and especially infrared spectrally sensitized silver halide emulsions. These compounds are also sensitizers for silver halide emulsions which are not spectrally sensitized. The supersensitizing compounds of the present invention may be generally represented by the formula:



wherein

Q is selected from N, P, As, Sb and Bi,

Ar is an aryl group, and

Ar' is an aryl group having a substituent thereon which renders the compound water-soluble.

Any aryl group, Ar, may be used in the practice of the present invention as long as the compound is water-soluble. The aryl group may be phenyl, naphthyl, thiophenyl, furanyl and pyrazolyl, for example. The aryl group, Ar, may be substituted or unsubstituted. The same substituents used on the aryl group, Ar', may be used or other substituents which do not prevent the compound from being water-soluble may be used. In addition to the substituents listed for Ar', such substituents as halogen (-Br, -Cl), nitro (-NO<sub>2</sub>), alcohols (-CH<sub>2</sub>OH), ethers (-CH<sub>2</sub>OCH<sub>3</sub>), amines (-N(alkyl)<sub>2</sub>), low molecular weight alkyls (CH<sub>3</sub>, CH<sub>2</sub>CH<sub>3</sub>) and the like may be used.

The aryl group, Ar', must bear at least one water-solubilizing substituent. Examples of highly efficient water-solubilizing substituents are sulfonates (with an associated cation such as alkali metal cations), sulfonic acid, sulfonic acid ester, carboxylate, carboxylic acid, carboxylic esters, alcohols (particularly low molecular weight alcohols of 1-3 carbons), phosphate, phosphite, phosphines, and nitro-compounds (i.e., -NO<sub>2</sub>). The strongly acidic members of that group are particularly preferred. Ar' may also be additionally substituted by groups that do not contribute positively to the water-solubility of the compounds, and more than one solubilizing group may be present on Ar'.

Examples of compounds of the present invention which are reported in the literature and/or commercially available include the following:

p-(Diphenylphosphino)benzoic acid  
Sodium diphenylphosphinobenzene-m-sulfonate  
Trisodium salt of tri-(m-sulfophenyl)arsine (trisodium triphenylarsine-m,m',m"-trisulfonate)

Tri-(m-[sulfonic acid]phenyl)arsine  
 Tri-(p-[methyl ester sulfonic acid]-phenyl)phosphine  
 m-(Diphenylphosphino)benzoic acid  
 (p-Carbomethoxyphenyl)diphenylphosphine  
 o-(Diphenylphosphino)benzoic acid  
 3,3'-(Phenylphosphinidene)di-benzoic acid 4,4'-  
 (Phenylphosphinidene)di-benzoic acid  
 2,2',2''-(Arylsilylidyne)tri-benzoic acid  
 4,4',4''-Phosphinidynetris-benzoic acid  
 3,3',3''-Phosphinidynetri-benzoic acid  
 2-(Diphenylarsino)benzoic acid  
 p-(Diphenylarsino)benzoic acid  
 p-(Diphenylarsino)methyl ester benzoic acid  
 3,3',3''-(Arylsilylidyne)tri-benzoic acid  
 4,4',4''-Stibylydinetris-benzoic acid  
 p-(Diphenylstibylydine)benzoic acid  
 p-(Diphenylstibylydine)sulfonic acid sodium salt  
 4,4',4''-Phosphinidynetris-benzoic acid trimethyl ester  
 2-(Diphenylamino)-5-methyl-1,3-benzenedicarboxylic  
 acid  
 2-[(2-Aminophenyl)phenylamino]benzoic acid  
 2-[(2-Nitrophenyl)phenylamino]benzoic acid  
 2-(Diphenylamino)benzoic acid  
 2-[(2,5-Dichlorophenyl)phenylamino]benzoic acid  
 2-[Bis(4-methylphenyl)arsino]benzoic acid  
 2,2',2''-Nitrilotris-benzene methanol triacetate  
 p-(Diphenylbismuthine)benzoic acid  
 2,2'-(Phenylbismuthine)dibenzoic acid  
 3,3',3''-Bismuthine-tris-benzoic acid  
 3,3',3''-Bismuthine-tris-sulfonic acid tri-sodium salt

The term "water-soluble" as used in the practice of the present invention indicates that the compound is soluble in an amount of at least 0.5 g/liter. Preferably the compound is soluble in an amount of at least 1 g/liter.

These type of compounds are added to the optically sensitized emulsions in any of the conventional methods by which supersensitizers or other adjuvants are added to photographic emulsions. Typically the water-soluble supersensitizing compounds of the present invention are added into the emulsion mixture just prior to coating, mixed well, then coated onto the photographic substrate. The compounds are added as aqueous solutions, alone, or with other desirable adjuvants.

The compounds of the present invention may be added in any effective supersensitizing amount to the photographic emulsion. The concentration of ingredients and materials can vary significantly in photographic emulsions such as from 0.5 to 10 g/m<sup>2</sup> for silver. The supersensitizers may also vary significantly in concentration. A generally useful range would be from 0.001 to 0.5 percent by dry weight of the total silver halide emulsion layer. This would generally comprise about 0.01 to 50% by weight of the silver halide in the photographic emulsion layer. A more preferred range would be from 0.1 to 3% by weight of the silver halide or about 0.01 to 0.3% total dry weight of the coated emulsion layer.

Any spectral sensitizing dye and any infrared spectral sensitizing dye may be used in the practice of the present invention with the water-soluble supersensitizing compounds of the present invention. Useful dyes for this purpose tend to be merocyanines, cyanines and especially tricarbocyanines. Such dye sensitizers for the infrared are described for example in U.S. Pat. Nos. 3,619,154, 3,682,630, 3,690,891, 3,695,888, 4,030,932 and 4,367,800. The preferred classes of compounds are the tricarbocyanines such as the 3,3'-dialkylthiatricarbocya-

nines, thiatricarbocyanines (especially with rigidized chains), selenotricarbocyanines, and enamine tricarbocyanines.

Silver halide emulsions supersensitized in accordance with this invention can comprise silver chloride, silver bromide, silver bromoiodide, silver chloroiodide, silver chlorobromoiodide or mixtures thereof. Such emulsions can be coarse, medium or fine grain (or mixtures thereof) and can be prepared by any of the well-known procedures, e.g., single jet emulsions or double jet emulsions. Useful emulsions include Lippmann emulsions, ammoniacal emulsions, thiocyanate or thioether ripened emulsions such as those described in Nietz et al., U.S. Pat. No. 2,222,264, Illingsworth, U.S. Pat. No. 3,320,069, and McBride, U.S. Pat. No. 3,271,157; or, cubic grain emulsions, such as those described by Kline and Moisar, Journal of Photographic Science, volume 12, page 242 et seq. or Markocki, The Spectral Sensitization of Silver Bromide Emulsions on Different Crystallographic Faces, Journal of Photographic Science, volume 13, 1965; or Illingsworth, British Pat. No. 1,156,193 published June 25, 1969.

Tabular or lamellar grain emulsions as described in U.S. Pat. Nos. 4,425,425 and 4,425,426 are also equally useful.

The silver halide emulsions supersensitized with the dyes of this invention can be unwashed or washed to remove soluble salts. In the latter case the soluble salts can be removed by chill-setting and leaching or the emulsion can be coagulation washed e.g., by the procedures described in Hewitson et al., U.S. Pat. No. 2,618,556; Yutzy et al., U.S. Pat. No. 2,614,928; Yackel, U.S. Pat. No. 2,565,418; Hart et al., U.S. Pat. No. 3,241,969; and Waller et al., U.S. Pat. No. 2,489,341.

Photographic emulsions containing supersensitizing combinations in accordance with this invention can be sensitized with chemical sensitizers, such as with reducing agents; sulfur, selenium or tellurium compounds; gold, platinum or palladium compounds; or combinations of these. Suitable chemical sensitization procedures are described in Shepard, U.S. Pat. No. 1,623,499; Waller, U.S. Pat. No. 2,399,083; McVeigh, U.S. Pat. No. 3,297,447; and Dunn, U.S. Pat. No. 3,297,446.

The supersensitized silver halide emulsions of this invention can contain speed increasing compounds such as polyalkylene glycols, cationic surface active agents and thioethers or combinations of these as described in Piper, U.S. Pat. No. 2,886,437; Chechak, U.S. Pat. No. 3,046,134; Carroll et al., U.S. Pat. No. 2,944,900; and Goffe, U.S. Pat. No. 3,294,540.

Silver halide emulsions containing the supersensitizing combinations of this invention can be protected against the production of fog and can be stabilized against loss of sensitivity during keeping. Suitable anti-foggants and stabilizers which can be used alone or in combination, include the thiazolium salts described in Staud, U.S. Pat. No. 2,131,038 and Allen, U.S. Pat. No. 2,694,716; the azaindenes described in Piper, U.S. Pat. No. 2,886,437 and Heimbach, U.S. Pat. No. 2,444,605; the mercury salts described in Allen, U.S. Pat. No. 2,728,663; the urazoles described in Anderson, U.S. Pat. No. 3,287,135; the sulfocatechols described in Kennard, U.S. Pat. No. 3,235,652; the oximes described in Carroll et al., British Pat. No. 623,448; nitron, nitroindazoles; the mercaptotetrazoles described in Kendall et al., U.S. Pat. No. 2,403,927, Kennard et al., U.S. Pat. No. 3,266,897 and Luckey et al., U.S. Pat. No. 3,397,987; the polyvalent metal salts described in Jones, U.S. Pat. No.

2,839,405; the thiuronium salts described in Herz, U.S. Pat. No. 3,220,839; and the palladium, platinum and gold salts described in Trivelli, U.S. Pat. No. 2,566,263 and Damschroder, U.S. Pat. No. 2,597,915.

Photographic elements including emulsions supersensitized in accordance with this invention can contain incorporated developing agents such as hydroquinones, catechols, aminophenols, 3-pyrazolidones, ascorbic acid and its derivatives, reductones and phenylenediamines, or combinations of developing agents. The developing agents can be in the silver halide emulsion and/or in another suitable location in the photographic element. The developing agents can be added from suitable solvents or in the form of dispersions as described in Yackel, U.S. Pat. No. 2,592,368 and Dunn et al., French Pat. No. 1,505,778.

Silver halide supersensitized in accordance with the invention can be dispersed in colloids that can be hardened by various organic or inorganic hardeners, alone or in combination, such as the aldehydes, and blocked aldehydes, ketones, carboxylic and carbonic acid derivatives, sulfonate esters, sulfonyl halides and vinyl sulfones, active halogen compounds, epoxy compounds, aziridines, active olefins, isocyanates, carbodiimides, mixed function hardeners and polymeric hardeners such as oxidized polysaccharides, e.g., dialdehyde starch, oxyguargum, etc.

Photographic emulsions supersensitized with the materials described herein can contain various colloids alone or in combination as vehicles or binding agents. Suitable hydrophilic materials include both naturally-occurring substances such as proteins, for example, gelatin, gelatin derivatives, (e.g., phthalated gelatin), cellulose derivatives, polysaccharides such as dextran, gum arabic and the like; and synthetic polymeric substances such as water soluble polyvinyl compounds, e.g., poly(vinylpyrrolidone)acrylamide polymers or other synthetic polymeric compounds such as dispersed vinyl compounds in latex form, and particularly those which increase the dimensional stability of the photographic materials. Suitable synthetic polymers include those described, for example, in U.S. Pat. Nos. 3,142,568 of Nottorf; 3,193,386 of White; 3,062,674 of Houck, Smith and Yudelson; 3,220,844 of Houck, Smith and Yudelson; Ream and Fowler, 3,287,289; and Dykstra, U.S. Pat. No. 3,411,911; particularly effective are those water-insoluble polymers of alkyl acrylates and methacrylates, acrylic acid, sulfoalkyl acrylates or methacrylates, those which have cross linking sites which facilitate hardening or curing and those having recurring sulfobentaine units as described in Canadian Pat. No. 774,054.

Emulsions supersensitized in accordance with this invention can be used in photographic elements which contain antistatic or conducting layers, such as layers that comprise soluble salts, e.g., chlorides, nitrates, etc., evaporated metal layers, ionic polymers such as those described in Minsk, U.S. Pat. Nos. 2,861,056 and 3,206,312 or insoluble inorganic salts such as those described in Trevoy, U.S. Pat. No. 3,428,451.

Photographic emulsions containing the supersensitizing combinations of the invention can be coated on a wide variety of supports. Typical supports include polyester film, subbed polyester film, poly(ethylene terephthalate) film, cellulose nitrate film, cellulose ester film, poly(vinyl acetal) film, polycarbonate film and related films or resinous materials, as well as glass, paper, metal and the like. Typically, a flexible support is

employed, especially a paper support, which can be partially acetylated or coated with baryta and/or an alpha-olefin polymer, particularly a polymer of an alpha-olefin containing 2 to 10 carbon atoms such as polyethylene, polypropylene, ethylenebutene copolymers and the like.

Supersensitized emulsions of the invention can contain plasticizers and lubricants such as polyalcohols, e.g., glycerin and diols of the type described in Milton, U.S. Pat. No. 2,960,404; fatty acids or esters such as those described in Robijns, U.S. Pat. No. 2,588,765 and Duane, U.S. Pat. No. 3,121,060; and silicone resins such as those described in DuPont British Pat. No. 955,061.

The photographic emulsions supersensitized as described herein can contain surfactants such as saponin, anionic compounds such as the alkylarylsulfonates described in Baldsiefen, U.S. Pat. No. 2,600,831 fluorinated surfactants, and amphoteric compounds such as those described in Ben-Ezra, U.S. Pat. No. 3,133,816.

Photographic elements containing emulsion layers sensitized as described herein can contain matting agents such as starch, titanium dioxide, zinc oxide, silica, polymeric beads including beads of the type described in Jelley et al., U.S. Pat. No. 2,992,101 and Lynn, U.S. Pat. No. 2,701,245.

Spectrally sensitized emulsions of the invention can be utilized in photographic elements which contain brightening agents including stilbene, triazine, oxazole and coumarin brightening agents. Water soluble brightening agents can be used such as those described in Albers et al., German Pat. No. 972,067 and McFall et al., U.S. Pat. No. 2,933,390 or dispersions of brighteners can be used such as those described in Jansen, German Pat. No. 1,150,274 and Oetiker et al., U.S. Pat. No. 3,406,070.

Photographic elements containing emulsion layers supersensitized according to the present invention can be used in photographic elements which contain light absorbing materials and filter dyes such as those described in Sawdey, U.S. Pat. No. 3,253,921; Gaspar, U.S. Pat. No. 2,274,782; Carroll et al., U.S. Pat. No. 2,527,583 and Van Campen, U.S. Pat. No. 2,956,879. If desired, the dyes can be mordanted, for example, as described in Milton and Jones, U.S. Pat. No. 3,282,699.

The sensitizing dyes and/or supersensitizers (and other emulsion addenda) can be added to the photographic emulsions from water solution or suitable organic solvent solutions, for example with the procedure described in Collins et al., U.S. Pat. No. 2,912,343; Owens et al., U.S. Pat. No. 3,342,605; Audran, U.S. Pat. No. 2,996,287 or Johnson et al., U.S. Pat. No. 3,425,835. The dyes can be dissolved separately or together, and the separate or combined solutions can be added to a silver halide emulsion, or a silver halide emulsion layer can be bathed in the solution of supersensitizers and/or dyes.

Contrast enhancing additives such as hydrazines, rhodium, iridium and combinations thereof are also useful.

Photographic emulsions of this invention can be coated by various coating procedures including dip coating, air knife coating, curtain coating, or extrusion coating using hoppers of the type described in Beguin, U.S. Pat. No. 2,681,294. If desired, two or more layers may be coated simultaneously by the procedures described in Russell, U.S. Pat. No. 2,761,791 and Wynn British Pat. No. 837,095.

Silver halide emulsions containing the supersensitizer combinations of this invention can be used in elements designed for color photography, for example, elements containing color-forming couplers such as those described in Frolich et al., U.S. Pat. No. 2,376,679; Vittum et al., U.S. Pat. No. 2,322,027; Fierke et al., U.S. Pat. No. 2,801,171; Godowsky, U.S. Pat. No. 2,698,794; Barr et al., U.S. Pat. No. 3,227,554 and Graham, U.S. Pat. No. 3,046,129; or elements to be developed in solutions containing color-forming couplers such as those described in Mannes and Godowsky, U.S. Pat. No. 2,252,718; Carroll et al. U.S. Pat. No. 2,592,243 and Schwan, U.S. Pat. No. 2,950,970.

Exposed photographic emulsions of this invention can be processed by various methods including processing in alkaline solutions containing conventional developing agents such as hydroquinones, catechols, aminophenols, 3-pyrazolidones, phenylenediamines, ascorbic acid derivatives, hydroxylamines, hydrazines and the like; web processing such as described in Tegillus et al., U.S. Pat. No. 3,179,517; stabilization processing as described in Yackel et al. "Stabilization Processing of Films and Papers", PSA Journal, vol. 16B, August 1950; monobath processing as described in Levy "Combined Development and fixation of Photographic Images with Monobaths", Phot. Sci. and Eng., vol. 2, No. 3, October 1958, and Barnes et al. U.S. Pat. No. 3,392,019. If desired, the photographic emulsions of this invention can be processed in hardening developers such as those described in Allen et al., U.S. Pat. No. 3,232,761; in roller transport processors such as those described in Russel, U.S. Pat. No. 3,025,779; or by surface application processing as described in Example 3, of Kitze, U.S. Pat. No. 3,418,132.

Particularly useful additives in the practice of the present invention which are effectively combined with the water-soluble supersensitizing compounds are poly(ethyl acrylate), phenylmercaptotetrazole and Leucophor BCF (hereinafter PEA, PMT and BCF, respectively).

These and other aspects of the invention will be shown by the Examples.

Two different emulsions are used in the various examples to show the practice of the present invention.

The emulsion was divided in half for two different types of chemical sensitization. Emulsion Aa was digested with sodium thiosulfate while Ab was digested with p-toluenesulfinic acid, sodium thiosulfate and sodium gold tetrachloride (NaAuCl<sub>4</sub>).

Final preparation of the emulsions comprised the addition of water and gelatin to a level of 5.0% gelatin and 2500 g of emulsion per mole of silver. The pH was adjusted to 7.0, and the pAg was adjusted to 7.2. Infrared sensitizing dyes were added as 0.04% by weight solutions in methanol. PMT was added as a 0.1% methanol solution and PEA as a 20% aqueous solution. The water-soluble supersensitizer, formaldehyde hardener and any other indicated materials were added before coating as an aqueous solution.

## EXAMPLES 1-20

The effect of various individual and combinations of additives on photographic silver halide emulsions were investigated. Emulsion Ab was dyed with the infrared sensitizing dye shown below, and diphenylphosphino-benzene-m-sulfonate sodium salt (DBS) was the water-soluble compound. The coated and dried film was aged one week before exposing on a sensitometer for 10<sup>-3</sup> seconds through a Huoy cut-off filter which filtered out all radiation below 760 nm. The exposed films were developed in a 90 second Xray processor. Sensitometric measurements include D<sub>min</sub>, D<sub>max</sub>, speed (at O.D.=0.25), average contrast (C̄), change in speed from emulsion without additives (dS), and the percent that change (ds) represented (% dS). The measurements were taken on the photographic element when freshly dried and on a sample incubated for three days at 50° C. and 40% R.H. The amounts of PMT, DBS, BCF and PEA are presented in grams per mole of silver. The results are shown in Table I for emulsion Ab.



TABLE I

| Ex | PMT   | DBS  | BCF  | PEA | Fresh |      |      | Incubated |      |      |      |      |
|----|-------|------|------|-----|-------|------|------|-----------|------|------|------|------|
|    |       |      |      |     | Dmin  | Dmax | S    | C̄        | dS   | % dS | Dmin | Dmax |
| 1  | 0     | 0    | 0    | 0   | 0.03  | 3.25 | 1.17 | 3.26      | —    | 100  | 0.04 | 3.18 |
| 2  | 0.038 | 0    | 0    | 0   | 0.03  | 3.30 | 1.40 | 3.23      | 0.23 | 170  | 0.04 | 3.22 |
| 3  | 0     | 0.28 | 0    | 0   | 0.03  | 3.28 | 1.45 | 2.86      | 0.28 | 190  | 0.04 | 3.24 |
| 4  | 0     | 0    | 0.50 | 0   | 0.04  | 3.32 | 2.01 | 3.13      | 0.84 | 692  | 0.05 | 3.25 |
| 5  | 0     | 0    | 0    | 30  | 0.03  | 3.17 | 1.36 | 3.31      | 0.19 | 155  | 0.04 | 3.14 |
| 6  | 0.038 | 0.28 | 0    | 0   | 0.03  | 3.20 | 1.38 | 2.82      | 0.21 | 162  | 0.04 | 3.18 |
| 7  | 0.038 | 0    | 0.50 | 0   | 0.04  | 3.41 | 1.91 | 3.20      | 0.74 | 550  | 0.04 | 3.17 |
| 8  | 0.038 | 0    | 0    | 30  | 0.03  | 3.25 | 1.66 | 3.21      | 0.49 | 309  | 0.04 | 3.21 |
| 9  | 0     | 0.28 | 0.50 | 0   | 0.04  | 3.28 | 1.94 | 2.83      | 0.77 | 589  | 0.05 | 3.22 |
| 10 | 0     | 0.28 | 0    | 30  | 0.03  | 3.17 | 1.58 | 2.80      | 0.41 | 257  | 0.04 | 3.16 |
| 11 | 0     | 0    | 0.50 | 30  | 0.03  | 3.38 | 2.07 | 3.20      | 0.90 | 794  | 0.04 | 3.19 |
| 12 | 0.038 | 0.28 | 0.50 | 0   | 0.03  | 3.31 | 1.86 | 2.84      | 0.69 | 490  | 0.04 | 3.20 |
| 13 | 0.038 | 0.28 | 0    | 30  | 0.03  | 3.15 | 1.60 | 2.77      | 0.43 | 269  | 0.04 | 3.12 |
| 14 | 0.038 | 0    | 0.50 | 30  | 0.03  | 3.20 | 2.10 | 3.18      | 0.91 | 851  | 0.04 | 3.07 |
| 15 | 0     | 0.28 | 0.50 | 30  | 0.03  | 3.24 | 2.00 | 2.86      | 0.83 | 676  | 0.04 | 3.04 |
| 16 | 0.038 | 0.28 | 0.50 | 30  | 0.03  | 3.12 | 1.97 | 2.74      | 0.80 | 631  | 0.04 | 3.13 |
| 17 | 0.019 | 0.14 | 0.25 | 15  | 0.03  | 3.24 | 1.96 | 2.99      | 0.79 | 617  | 0.04 | 3.15 |
| 18 | 0.019 | 0.14 | 0.25 | 15  | 0.04  | 3.21 | 1.96 | 2.95      | 0.79 | 617  | 0.04 | 3.20 |
| 19 | 0.019 | 0.14 | 0.25 | 15  | 0.03  | 3.15 | 1.96 | 2.90      | 0.79 | 617  | 0.04 | 3.16 |
| 20 | 0.019 | 0.14 | 0.25 | 15  | 0.03  | 3.24 | 1.96 | 2.96      | 0.79 | 617  | 0.04 | 3.12 |

Emulsion A was prepared by a double jet precipitation to provide an emulsion with 64% chloride and 36% bromide with an average grain size of 0.24 micrometers.

The data show that DBS is an efficient supersensitizer. DBS works very effectively in combination with

each and every additive of phenylmercaptotetrazole, poly(ethylacrylate), and Leucophor BCF.

## EXAMPLES 21-40

Examples 1-20 were repeated on emulsion Ab except that the infrared spectral sensitizing dye:

## EXAMPLE 61-69

Emulsion Ab was used with 15.0 grams PEA per mole of silver and 75 ml of a 0.04% by weight methanol solution of the following infrared sensitizing dyes:



was used. The results are reported in Table II.

TABLE II

| Ex | PMT   | DBS  | BCF  | PEA | Dmin | Dmax | S    | $\bar{C}$ | dS   | % dS | Incubated |      |      |           |      |
|----|-------|------|------|-----|------|------|------|-----------|------|------|-----------|------|------|-----------|------|
|    |       |      |      |     |      |      |      |           |      |      | Dmin      | Dmax | S    | $\bar{C}$ | -dS  |
| 21 | 0     | 0    | 0    | 0   | 0.04 | 3.31 | 1.41 | 3.19      | —    | 100  | 0.05      | 3.27 | 1.39 | 3.03      | 0.02 |
| 22 | 0.038 | 0    | 0    | 0   | 0.04 | 3.38 | 1.80 | 3.22      | 0.39 | 245  | 0.05      | 3.27 | 1.68 | 2.90      | 0.12 |
| 23 | 0     | 0.28 | 0    | 0   | 0.04 | 3.36 | 1.65 | 2.87      | 0.24 | 174  | 0.05      | 3.27 | 1.54 | 2.66      | 0.11 |
| 24 | 0     | 0    | 0.50 | 0   | 0.04 | 3.38 | 1.67 | 3.17      | 0.26 | 182  | 0.05      | 3.25 | 1.54 | 2.89      | 0.13 |
| 25 | 0     | 0    | 0    | 30  | 0.04 | 3.31 | 1.55 | 3.18      | 0.14 | 138  | 0.05      | 3.21 | 1.52 | 2.93      | 0.03 |
| 26 | 0.038 | 0.28 | 0    | 0   | 0.04 | 3.35 | 1.73 | 2.88      | 0.32 | 209  | 0.05      | 3.22 | 1.63 | 2.76      | 0.10 |
| 27 | 0.038 | 0    | 0.50 | 0   | 0.04 | 3.38 | 1.76 | 3.16      | 0.36 | 229  | 0.05      | 3.31 | 1.64 | 2.96      | 0.12 |
| 28 | 0.038 | 0    | 0    | 30  | 0.04 | 3.40 | 1.86 | 3.29      | 0.45 | 282  | 0.05      | 2.09 | 1.73 | 2.89      | 0.13 |
| 29 | 0     | 0.28 | 0.50 | 0   | 0.04 | 3.37 | 1.84 | 2.93      | 0.43 | 269  | 0.05      | 3.31 | 1.73 | 2.76      | 0.11 |
| 30 | 0     | 0.28 | 0    | 30  | 0.04 | 3.27 | 1.80 | 2.90      | 0.39 | 245  | 0.05      | 3.16 | 1.74 | 2.75      | 0.06 |
| 31 | 0     | 0    | 0.50 | 30  | 0.04 | 3.20 | 1.90 | 3.07      | 0.49 | 309  | 0.05      | 3.22 | 1.84 | 2.96      | 0.06 |
| 32 | 0.038 | 0.28 | 0.50 | 0   | 0.04 | 3.44 | 1.83 | 2.98      | 0.42 | 263  | 0.05      | 3.38 | 1.73 | 2.78      | 0.10 |
| 33 | 0.038 | 0.28 | 0    | 30  | 0.04 | 3.40 | 1.86 | 2.92      | 0.45 | 282  | 0.05      | 3.24 | 1.79 | 2.70      | 0.07 |
| 34 | 0.038 | 0    | 0.50 | 30  | 0.04 | 3.33 | 1.96 | 3.16      | 0.55 | 355  | 0.05      | 3.17 | 1.88 | 2.98      | 0.08 |
| 35 | 0     | 0.28 | 0.50 | 30  | 0.04 | 3.19 | 1.97 | 2.83      | 0.56 | 363  | 0.05      | 3.19 | 1.92 | 2.72      | 0.05 |
| 36 | 0.038 | 0.28 | 0.50 | 30  | 0.04 | 3.28 | 1.98 | 2.84      | 0.57 | 372  | 0.04      | 3.15 | 1.90 | 2.66      | 0.08 |
| 37 | 0.019 | 0.14 | 0.25 | 15  | 0.04 | 3.18 | 1.86 | 2.95      | 0.45 | 282  | 0.05      | 3.24 | 1.78 | 2.87      | 0.08 |
| 38 | 0.019 | 0.14 | 0.25 | 15  | 0.04 | 3.37 | 1.87 | 3.07      | 0.46 | 288  | 0.04      | 3.20 | 1.76 | 2.84      | 0.11 |
| 39 | 0.019 | 0.14 | 0.25 | 15  | 0.04 | 3.38 | 1.87 | 3.11      | 0.46 | 288  | 0.05      | 3.25 | 1.77 | 2.88      | 0.10 |
| 40 | 0.019 | 0.14 | 0.25 | 15  | 0.04 | 3.31 | 1.88 | 3.06      | 0.47 | 295  | 0.05      | 3.31 | 1.74 | 2.91      | 0.11 |

## EXAMPLES 41-60

Examples 21-40 were repeated except that Emulsion Aa was used with the same infrared sensitizing dye. The results are reported in Table III.



b.

TABLE III

| Ex | PMT   | DBS  | BCF  | PEA | Dmin | Dmax | S    | $\bar{C}$ | dS   | % dS | Incubated |      |      |           |      |
|----|-------|------|------|-----|------|------|------|-----------|------|------|-----------|------|------|-----------|------|
|    |       |      |      |     |      |      |      |           |      |      | Dmin      | Dmax | S    | $\bar{C}$ | -dS  |
| 41 | 0     | 0    | 0    | 0   | 0.04 | 3.67 | 1.32 | 2.38      | —    | 100  | 0.04      | 3.55 | 1.30 | 2.25      | 0.02 |
| 42 | 0.038 | 0    | 0    | 0   | 0.04 | 3.90 | 1.58 | 2.41      | 0.26 | 182  | 0.04      | 3.74 | 1.52 | 2.26      | 0.06 |
| 43 | 0     | 0.28 | 0    | 0   | 0.03 | 3.59 | 1.40 | 2.04      | 0.08 | 120  | 0.04      | 3.47 | 1.35 | 1.99      | 0.05 |
| 44 | 0     | 0    | 0.50 | 0   | 0.04 | 3.88 | 1.57 | 2.37      | 0.25 | 179  | 0.04      | 3.67 | 1.50 | 2.30      | 0.07 |
| 45 | 0     | 0    | 0    | 30  | 0.04 | 3.59 | 1.37 | 2.41      | 0.05 | 112  | 0.04      | 3.43 | 1.35 | 2.28      | 0.02 |
| 46 | 0.038 | 0.28 | 0    | 0   | 0.03 | 3.64 | 1.45 | 2.03      | 0.13 | 135  | 0.04      | 3.54 | 1.42 | 2.04      | 0.03 |
| 47 | 0.038 | 0    | 0.50 | 0   | 0.04 | 3.88 | 1.62 | 2.39      | 0.30 | 200  | 0.04      | 3.73 | 1.54 | 2.21      | 0.08 |
| 48 | 0.038 | 0    | 0    | 30  | 0.04 | 3.84 | 1.58 | 2.51      | 0.26 | 182  | 0.04      | 3.50 | 1.55 | 2.37      | 0.03 |
| 49 | 0     | 0.28 | 0.50 | 0   | 0.04 | 3.82 | 1.64 | 2.11      | 0.32 | 209  | 0.04      | 3.71 | 1.57 | 2.00      | 0.07 |
| 50 | 0     | 0.28 | 0    | 30  | 0.03 | 3.69 | 1.54 | 2.05      | 0.22 | 166  | 0.03      | 3.47 | 1.50 | 1.97      | 0.04 |
| 51 | 0     | 0    | 0.50 | 30  | 0.04 | 3.92 | 1.73 | 2.44      | 0.41 | 257  | 0.04      | 3.63 | 1.65 | 2.16      | 0.08 |
| 52 | 0.038 | 0.28 | 0.50 | 0   | 0.04 | 3.73 | 1.59 | 2.05      | 0.27 | 186  | 0.04      | 3.67 | 1.53 | 2.02      | 0.06 |
| 53 | 0.038 | 0.28 | 0    | 30  | 0.03 | 3.67 | 1.57 | 2.06      | 0.25 | 179  | 0.03      | 3.49 | 1.50 | 1.94      | 0.07 |
| 54 | 0.038 | 0    | 0.50 | 30  | 0.04 | 3.85 | 1.77 | 2.36      | 0.45 | 282  | 0.04      | 3.66 | 1.70 | 2.25      | 0.07 |
| 55 | 0     | 0.28 | 0.50 | 30  | 0.03 | 3.68 | 1.70 | 2.01      | 0.38 | 240  | 0.03      | 3.54 | 1.64 | 1.92      | 0.06 |
| 56 | 0.038 | 0.28 | 0.50 | 30  | 0.03 | 3.68 | 1.66 | 2.01      | 0.34 | 219  | 0.03      | 3.52 | 1.62 | 1.93      | 0.04 |
| 57 | 0.019 | 0.14 | 0.25 | 15  | 0.03 | 3.84 | 1.66 | 2.17      | 0.34 | 219  | 0.04      | 3.64 | 1.60 | 2.09      | 0.06 |
| 58 | 0.019 | 0.14 | 0.25 | 15  | 0.03 | 3.82 | 1.66 | 2.16      | 0.34 | 219  | 0.04      | 3.65 | 1.60 | 2.10      | 0.06 |
| 59 | 0.019 | 0.14 | 0.25 | 15  | 0.03 | 3.79 | 1.64 | 2.15      | 0.32 | 209  | 0.03      | 3.58 | 1.57 | 2.06      | 0.07 |
| 60 | 0.019 | 0.14 | 0.25 | 15  | 0.03 | 3.80 | 1.63 | 2.16      | 0.31 | 204  | 0.03      | 3.68 | 1.59 | 2.12      | 0.04 |



The results are reported in Table IV for fresh samples exposed at 10<sup>-3</sup> seconds through an 810 nm, narrow band filters. The speed values at O.D.=1.0 (S<sub>1</sub>) and O.D.=0.25 (S<sub>2</sub>) were measured.

TABLE IV

| Ex. | Dye | Add. | D <sub>min</sub> | D <sub>max</sub> | S <sub>1</sub> | S <sub>2</sub> | $\bar{C}$ |
|-----|-----|------|------------------|------------------|----------------|----------------|-----------|
| 61  | a   | —    | 0.03             | 3.49             | 2.26           | 1.94           | 3.00      |
| 62  | a   | DBS  | 0.03             | 3.31             | 2.40           | 2.03           | 2.54      |
| 63  | b   | —    | 0.04             | 3.27             | 1.84           | 1.51           | 2.87      |
| 64  | b   | DBS  | 0.04             | 3.13             | 1.96           | 1.61           | 2.69      |
| 65  | c   | —    | 0.03             | 3.33             | 1.79           | 1.48           | 3.02      |
| 66  | c   | DBS  | 0.03             | 3.32             | 2.10           | 1.74           | 2.49      |
| 67  | d   | —    | 0.03             | 3.24             | 1.62           | 1.27           | 2.81      |
| 68  | d   | DBS  | 0.03             | 3.18             | 1.75           | 1.37           | 2.53      |
| 69  | I   | DBS  | 0.03             | 3.31             | 2.63           | 2.26           | 2.58      |

## EXAMPLE 70

The addition of the following compounds in the same manner as the sodium diphenylphosphinobenzene-m-sulfonate of earlier examples also will show varying supersensitizing effects:

- 1. 2-(diphenylamino)benzoic acid
- 2. 4-(diphenylphosphino)benzoic acid
- 3. 4-(diphenylarsino)benzoic acid
- 4. Trisodium salt of tri-(m-sulfophenyl)arsine
- p-Diphenylbismuthinestris-sulfonic acid trisodium salt.

treated with post sensitization additives and stabilizers, namely tetraazainidines, additional halides, and conventional antifoggants, etc., as required and as is known in the art. The emulsion was coated to provide a silver coating weight in the range of 5.5 to 7.0 g/m<sup>2</sup>.

Emulsion B was divided into two portions. To the first portion was added PEA and varying amounts of DBS (Table V). The coated and dried material was evaluated with a 1/10 second exposure from a tungsten light source with a color temperature of 2650° K. The light was filtered with a Corning 5850 blue filter. The exposed films were developed in a 90 second X-ray processor, and the results are listed in Table V.

TABLE V

| Ex. | PEA | DBS   | Blue Filter      |                  |                  |      |
|-----|-----|-------|------------------|------------------|------------------|------|
|     |     |       | D <sub>min</sub> | D <sub>max</sub> | SPD <sub>2</sub> | AVCO |
| 71  | 25  | 0     | 0.18             | 3.19             | 1.96             | 3.10 |
| 72  | 25  | 0.014 | 0.19             | 3.09             | 1.98             | 3.01 |
| 73  | 25  | 0.035 | 0.19             | 3.16             | 2.03             | 3.04 |
| 74  | 25  | 0.070 | 0.19             | 3.26             | 2.06             | 3.01 |

The data verifies that DBS acts as a supersensitizer without the addition of spectral sensitizing dyes.

The second portion of Emulsion B was treated in the same manner as in Examples 71-74 with the exception that a green sensitizing dye (shown below) was added.



The films were evaluated as in Examples 71-74. In addition, a green filter system was substituted for the blue filter. The green filter was a narrow band interference filter centered at 546.1 nm. The results are shown in Table VI.

TABLE VI

| Ex | PEA | DBS   | Blue Filter      |                  |                  |      | Green Filter     |                  |                  |      |
|----|-----|-------|------------------|------------------|------------------|------|------------------|------------------|------------------|------|
|    |     |       | D <sub>min</sub> | D <sub>max</sub> | SPD <sub>2</sub> | AVCO | D <sub>min</sub> | D <sub>max</sub> | SPD <sub>2</sub> | AVCO |
| 5  | 25  | 0     | 0.19             | 3.54             | 1.96             | 3.08 | 0.19             | 3.49             | 2.02             | 3.09 |
| 6  | 25  | 0.007 | 0.19             | 3.59             | 1.99             | 3.12 | 0.19             | 3.52             | 2.04             | 3.09 |
| 7  | 25  | 0.035 | 0.19             | 3.55             | 2.02             | 3.07 | 0.19             | 3.52             | 2.08             | 3.06 |
| 8  | 25  | 0.140 | 0.22             | 3.54             | 2.10             | 2.94 | 0.22             | 3.52             | 2.12             | 2.94 |

## EXAMPLES 71-78

## Preparation of Emulsion B

Silver halide light sensitive Emulsion B was prepared by precipitation and ripening steps using 98.0 mole percent silver bromide and 2.0 mole percent silver iodide in the presence of 15 g gelatin per mole of silver halide. The precipitated silver halide was freed of unwanted soluble by-product salts by coagulation and washing using the method disclosed in U.S. Pat. No. 2,489,341 wherein the silver halide and most of the gelatin were coagulated by sodium lauryl sulfate, using an acid coagulation environment. Following the washing step, the emulsion coagulum was redispersed in water together with 67 g of additional gelatin. This redispersed emulsion was treated with conventional sulfur and gold sensitizers and was digested at 55° C. to increase sensitivity, was cooled to 40° C., and was then

55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060



where  $R^1$  and  $R^2$  are alkyl of 1 to 4 carbon atoms and  $X^-$  is any anion. The benzo groups may bear any photographically acceptable substituents, such as for example, alkyl (e.g., methyl, ethyl, propyl, butyl), alkoxy (e.g., methoxy, ethoxy, propoxy, butoxy), halogen (e.g., chlorine, bromine, iodine), amine (primary, secondary, tertiary aliphatic or aromatic amines), nitro, cyano, aryl (e.g. phenyl, naphthyl), fused on aromatic rings (e.g., to form naphthothiazoles), and mixtures of these groups. For example, 5-alkyl-6-alkoxy-, 5,6-dialkyl-, 5-alkoxy-6-alkyl, and 5,6-dialkoxy-benzothiazole terminal groups are preferred, particularly with  $C_1-C_4$  alkyl and alkoxy groups, and 5-methyl-6-methoxy is most preferred.

I claim:

1. A silver halide photographic emulsion in a hydrophilic colloidal binder, said emulsion being spectrally sensitized by a spectral sensitizing dye to at least a portion of the electromagnetic spectrum and having a supersensitizing amount of a water-soluble triaryl compound selected from the group consisting of phosphines, amines, arsines, bismuthines and stibylidynes.

2. The emulsion of claim 1 wherein at least one aryl group on said compounds has a water-solubilizing group selected from the class consisting of sulfonic acid, sulfonate, sulfonic acid salt, phosphate, phosphonate, carboxylic acid, carboxylic acid salt, carboxylate, alcohol, nitro-, and amine.

3. The emulsion of claim 1 wherein said compound is represented by the structural formula



wherein

$Q$  is selected from N, P, As, Sb and Bi,

$Ar$  is an aryl group, and

$Ar'$  is an aryl group bearing at least one substituent which renders said compound water-soluble.

4. The emulsion of claim 1 wherein  $Ar$  and  $Ar'$  are selected from phenyl groups.

5. The emulsion of claim 1 wherein at least one water-solubilizing substituent on  $Ar'$  is selected from the group consisting of sulfonic acid, sulfonic acid salt, sulfonate, carboxylic acid, carboxylic acid salt, carbox-

60

ylate, phosphate, phosphonate, alcohol, nitro- and amine.

6. The emulsion of claim 3 wherein the at least one water-solubilizing group on  $Ar'$  is selected from the group consisting of sulfonic acid, sulfonic acid salt, sulfonate, carboxylic acid, carboxylic acid salt and carboxylate.

7. The emulsion of claim 1 further comprising a supersensitizing amount of poly(ethylacrylate).

10 8. The emulsion of claim 4 further comprising a supersensitizing amount of poly(ethylacrylate).

9. The emulsion of claim 6 further comprising a supersensitizing amount of poly(ethylacrylate).

15 10. The emulsion of claim 1 further comprising a supersensitizing amount of phenylmercaptotetrazole.

11. The emulsion of claim 8 further comprising a supersensitizing amount of phenylmercaptotetrazole.

12. The emulsion of claim 9 further comprising a supersensitizing amount of phenylmercaptotetrazole.

20 13. The emulsion of claim 1 further comprising a supersensitizing amount of Leucophor BCF.

14. The emulsion of claim 4 further comprising a supersensitizing amount of Leucophor BCF.

15 15. The emulsion of claim 12 further comprising a supersensitizing amount of Leucophor BCF.

16. The emulsion of claim 6 wherein  $Ar$  and  $Ar'$  comprise phenyl groups, and there is present in the emulsion a supersensitizing amount of at least one compound selected from the group consisting of phenylmercaptotetrazole, poly(ethylacrylate), and Leucophor BCF.

30 17. The emulsion of claim 6 wherein  $Ar$  and  $Ar'$  comprise phenyl groups and  $Q$  is selected from the group consisting of P and As.

18. The emulsion of claim 17 wherein  $Q$  is P.

19. The emulsion of claim 4 wherein  $Q$  is P and the emulsion is spectrally sensitized to the infrared region of the electromagnetic spectrum.

40 20. The emulsion of claim 18 wherein the emulsion is a chlorobromide emulsion.

21. A silver halide photographic emulsion in a hydrophilic colloidal binder, said emulsion being spectrally sensitized by a spectral sensitizing dye to at least a portion of the electromagnetic spectrum and having a supersensitizing amount of a water-soluble triaryl compound selected from the group consisting of amines, arsines, bismuthines and stibylidynes.

45 22. The emulsion of claim 21 wherein at least one aryl group on said compounds has a water-solubilizing group selected from the class consisting of sulfonic acid, sulfonate, sulfonic acid salt, phosphate, phosphonate, carboxylic acid, carboxylic acid salt, carboxylate, alcohol, nitro-, and amine.

23. The emulsion of claim 21 further comprising a super-sensitizing amount of poly(ethylacrylate).

24. The emulsion of claim 21 further comprising a super-sensitizing amount of phenylmercaptotetrazole.

25. The emulsion of claim 21 further comprising a super-sensitizing amount of Leucophor BCF.

\* \* \* \* \*